

June 13, 1944.

W. R. COLLINGS

2,350,987

METHOD OF MAKING HIGHLY GLAZED FILM COATINGS

Filed April 27, 1942



Fig. 1



Fig. 2

INVENTOR.  
William R. Collings

BY

Griswold & Burdick  
ATTORNEYS

## UNITED STATES PATENT OFFICE

2,350,987

METHOD OF MAKING HIGHLY GLAZED  
FILM COATINGSWilliam R. Collings, Midland, Mich., assignor to  
The Dow Chemical Company, Midland, Mich.,  
a corporation of Michigan

Application April 27, 1942, Serial No. 440,573

7 Claims. (CL. 117—86)

This invention relates to an improved and continuous process for forming smooth, highly glazed finishing coatings of film forming substances, particularly of cellulose ethers, upon the surface of previously coated paper or other flexible sheet material.

It has long been desired to produce smooth, highly glazed surface coatings having an apparent optical depth on paper and other flexible sheet material, such as fabrics made from natural or synthetic fibers, sheets made from synthetic resins, cellulose derivatives, etc., but this has not heretofore been commercially feasible except in a few instances because of the relatively large amount of coating material required when using known processes and because of the expensive nature of the operation required to produce such surfaces. The usual methods of producing a highly glazed finish on such flexible sheets has heretofore involved the so-called "plate finishing" operation. In this operation the coated sheets are placed between polished plates of stainless steel, nickel or copper and subjected to high pressure in a press or between the rollers of a "plating" machine. This is a slow and expensive process which requires much handling of the sheet and the use of special presses, particularly if large sheets are desired. It is frequently necessary to heat the coated sheet to soften the coating material, and this may lead to the tendering of organic fibers. Furthermore, the method cannot be adapted readily to continuous operation. It is known that film-forming materials will produce a shiny appearance when coated on paper and other flexible fibrous sheets by conventional coating methods, such as by spraying, rolling, or doctoring a solution of the coating material in a volatile solvent onto the sheet and subsequently drying the coated sheet or by the methods of U. S. Patents 2,175,125 and 2,169,288; but to produce a smooth surface of good appearance and apparent optical depth a relatively thick coating of the film-forming material is usually required. To overcome these difficulties lamination of pre-cast films on the surface of the flexible sheet has in some cases been practiced but the coating is then often of such thickness that the coated product cannot readily be adapted to many commercial uses because of its stiffness.

It is accordingly an object of the present invention to provide an economical and continuous method for applying thin, uniform, glazed surface coatings to previously coated flexible sheets.

An additional object of the invention is to provide a compositely coated flexible sheet, the surface coating of which is smooth, highly glazed, and which has the appearance of great optical depth. An additional object is to provide a method whereby highly glazed coatings may be applied to flexible sheet material without involv-

ing excessively long drying of the coated sheet.

According to the present invention the foregoing and related objects are readily accomplished by first coating a flexible sheet in any convenient manner with a base coating of a plastic film-forming material, drying the coated sheet and applying to the dry coated sheet a thin finishing coat of a film-forming material in the manner hereinafter described. The finishing coat is applied by depositing a layer of a solution of the coating material in a volatile solvent on a polished surface, preferably on a polished roll or drum or on a traveling polished metal belt if continuous operation is desired, partially drying the deposited layer, pressing the dry previously coated flexible sheet onto the partially dried, tacky, cementitious layer of coating material while the latter is still on the polished surface, and subsequently stripping the compositely coated sheet from the polished surface.

For visual illustration of one mode in which the invention may be carried out, reference is had to the accompanying drawing wherein:

Fig. 1 is a diagrammatic elevation of apparatus in which the invention may be carried out; and

Fig. 2 is an enlarged diagrammatic cross-section, exaggerated in certain respects, of a coated sheet made by the method of the invention.

Referring to Fig. 1, a thin, uniform layer of a solution of a cellulose ether or other film-forming substance in a volatile solvent is cast from a hopper 3 onto the polished surface of a heated (heating means not shown) revolving metal drum 4 in such quantity as to form a thin film 5 thereon.

A dry previously coated flexible sheet 6 is drawn directly from a supply roll 7 or from the dry end of a conventional coating machine and its coated surface is pressed by means of a roll 8 into contact with the thin film 5 on the drum 4, while the film is still sufficiently wet with solvent to be of a tacky, non-self-supporting, adhesive consistency. The roll 8 is so positioned and tensioned that it exerts a firm pressure on the coated sheet and the finishing film between it and the drum 4. The roll and the drum are rotated at the same peripheral speed. The roll may be adjusted by means not shown to permit control of the distance the finishing film cast from the hopper is carried on the surface of the drum before it meets the coated flexible sheet. This furnishes one method of controlling the consistency of the film on the surface of the drum before it meets the coated flexible sheet. The surface temperature and peripheral speed of the drum may also

be adjusted to assist in controlling the consistency of the film. As the metal drum 4 rotates, the flexible sheet with the formed composite coating thereon is carried along with it and is stripped from it at a point ahead of the hopper 3. Although a certain amount of drying of the com-

posite coating occurs on the drum, it appears that the principal effect is the penetration of sufficient of the solvent remaining in the relatively thin finishing coat into the relatively thick base coat to enable the sheet bearing the composite coating to be stripped from the polished surface of the drum without distorting or disrupting the film surface. The coated and highly glazed sheet is then passed through a dryer 8 and the dried sheet wound on a roll 10 for storing or used continuously in a subsequent operation.

Referring now to Fig. 2, a flexible sheet 12 which may be of paper or sheets formed from natural or synthetic fibers, or the like coated on one side in a previous operation with a base coating 13 is shown after application of a highly glazed finishing coat 14 by the method of the present invention. The thickness of the flexible sheet and coating layers are shown greatly exaggerated for the sake of clarity. The finishing coat 14 has a smooth, highly glazed surface and is firmly adherent to the base coating 13.

Although any flexible sheet material, such as sheets composed of cotton, wool, silk, or other natural or synthetic fibers may be coated and then glazed by the method of the present invention, the invention has been found of particular value in the application of a highly glazed surface coating to previously coated paper stock. The finishing coat is preferably composed of the same material as the base coating, although it may be composed of any material which will adhere to the base coating and which is soluble in a solvent in which the material of the base coating is soluble. Thus, paper or other sheet material may be readily coated with ethyl cellulose dissolved in solvents and applied in known manner and, after drying, the coated sheet may be glazed by applying to it a very thin layer of ethyl cellulose dissolved in the same or similar solvents. If desired, the finishing coat may be of a harder and more abrasion resistant ethyl cellulose than that used to form the base coating, thus imparting to the coated article these desirable surface characteristics.

The degree of drying of the finishing coat which is effected on the polished surface before it is applied to the coated flexible sheet will vary considerably with the nature of the material being applied, the thickness of the finishing coat desired and with other factors. Usually the film is dried sufficiently on the polished surface so that it has a semisolid consistency, but is still tacky, non-self-supporting, cementitious, and incapable of being stripped from the polished surface. The thickness of the finishing coat applied to the coated flexible sheet may be varied over wide limits. Usually, unless it is desired to materially increase the total thickness of the coating on the sheet, a finishing coat between 0.05 and 2.0 mils thick will be found advantageous. It is usually desirable to apply a finishing coat which is relatively thin with respect to the base coating since, as mentioned above, it appears that the solvent remaining in the finishing coat when it meets the base coating almost immediately diffuses into the latter and is distributed substantially uniformly throughout the composite coating thus permitting satisfactory stripping of the coated sheet from the polished surface without the necessity of a long drying period. Finishing films from about 5 per cent to about 20 per cent of the thickness of the base coating may be satisfactorily applied in most cases without interfering with the stripping of

the coated sheet from the polished surface. Thicker finishing coats may, of course, be applied in which case additional drying of the composite film before it is stripped from the polished surface may be desirable. An influencing factor is, of course, the proportion of the solvent remaining in the finishing film when it comes in contact with the base coating on the flexible sheet. The maximum amount of solvent which may be present in the composite coating and still permit the coated sheet to be stripped from the polished surface will depend to some extent upon the nature and material of the polished surface and upon the material of which the finishing coat is composed. It is usually desirable, however, that the total amount of volatile solvent in the composite coating be less than 25 per cent, and preferably between 3 per cent and 20 per cent of the weight of the coating.

To facilitate removal of the coated sheet from the polished surface, it is often desirable to add to the solution, from which the finishing film is cast, small amounts of a stripping agent or of a substance which acts as a lubricant to prevent sticking of the finishing coat to the polished surface. Examples of compounds which have been tested and found suitable for this purpose include stearic acid, glycerol monostearate, triisopropanol amine and amine salts of higher fatty acid.

The subsequent drying operation after the compositely coated sheet is stripped from the polished surface may be carried out in any convenient manner, such as by blowing hot air over the coated sheet. Since the actual amount of solvent present is very small, the drying is accomplished rapidly.

The following example illustrates the practice of the invention, but it is not to be construed as limiting the scope thereof:

#### Example 1

A coating solution is prepared having the composition:

|                                             | Parts by weight |
|---------------------------------------------|-----------------|
| Ethyl cellulose (57 cps. type) <sup>1</sup> | 80              |
| Di-(ortho-xenyl) monophenyl phosphate       | 20              |
| Benzene                                     | 210             |
| Methanol                                    | 86              |

<sup>1</sup> Ethyl cellulose viscosity determined on a 5% solution by weight in a mixture of 80 parts by volume of toluene and 20 parts of ethanol.

The solution has a viscosity of about 120 seconds, measured by the falling ball method as described in the American Society for Testing Materials Standards for 1933; D-301-33 (p. 720). Paper is coated by the method of U. S. Patent 2,175,125 with a layer of this solution in amount sufficient to form a film having a thickness when dry of about 0.4 mil. The coated paper is dried and passed in continuous manner through the coating machine illustrated in Fig. 1. The polished steel drum is 4 feet in diameter and is heated to a temperature of 100°-110° C. A solution consisting of 20 per cent by weight of ethyl cellulose (150 cps. type), together with 0.2 per cent of stearic acid in a mixture of 80 parts by volume of toluene and 20 parts of methanol, is deposited from the hopper on the surface of the rotating drum in such quantities that it forms, when dry, a film about 0.1 mil thick. The dry coated side of the paper is pressed smoothly against the partially dried film on the drum, and the two are kept in contact for the greater part of one revolution of the drum. The assembly is then

stripped from the drum and is conducted through a drying chamber to complete the drying operation. The coating, which has a total thickness of about 0.5 mil, has a smooth, highly polished surface, and has the appearance of being much thicker than it actually is.

While the example given above illustrates the invention as applied to formation of a highly polished surface coating of ethyl cellulose on paper, the invention can be applied with equal advantage to formation of finishing films of other film-forming materials, such as water-soluble methyl cellulose, organo-soluble methyl cellulose, benzyl cellulose, salts of cellulose glycolic acid, cellulose acetate, cellulose nitrate, acrylic acid ester polymers, etc., on other flexible, coated sheets, such as coated cotton, wool or silk cloth, rayon, etc. The process may also be used to apply a surface coating to a precast plastic film to give the latter improved surface characteristics. Flexible coated sheets may be glazed on each side by first glazing one side of the sheet and then, after turning it over, glazing the other side. In its broader aspects the invention concerns a continuous process for forming smooth highly glazed surface coatings on flexible coated sheet materials. In its practical application the invention is limited in its scope only by the requirement that the ingredients of the film forming substances used in the base coating and in the finishing coat be soluble in the same solvent and capable of adhering to each other.

Among the advantages of the invention may be mentioned the following: (1) the coating may be applied rapidly and economically, (2) the coating applied by the process of the invention improves the surface characteristics of the coated sheet and provides a uniform appearance, (3) the composite coating gives the desirable impression of apparent optical depth to ink imprints on the flexible sheet material beneath the coating which it has been impossible to obtain heretofore except by lamination methods using thicker films than are necessary in carrying out the present invention, and (4) it provides a method whereby finishing coats may be applied to flexible sheets without the use of long drying periods.

I claim:

1. The method which includes: depositing a uniform thin layer of a solution of a film-forming substance in a volatile solvent on a polished metal surface; partially drying the solution on the polished surface; superposing and pressing thereon a dry coated face of a flexible sheet coated on at least one side with a film soluble in the said volatile solvent and adapted to adhere to the said film-forming substance; stripping the compositely coated sheet from the polished surface; and drying the coated sheet.

2. The method which includes: depositing a uniform thin layer of a solution of a cellulose ether in a volatile solvent on a polished metal surface; partially drying the solution on the polished surface; superposing and pressing thereon a dry coated face of a flexible sheet coated on at least one side with a cellulose ether soluble in the said volatile solvent; and stripping the compositely coated sheet from the polished surface.

3. The method which includes: depositing a uniform layer of a solution of a cellulose ether in

a volatile solvent on a polished metal surface in amount sufficient to form a relatively thin film thereon upon evaporation of the solvent; partially drying the solution on the polished surface; superposing and pressing thereon a dry coated face of a flexible sheet coated on at least one side with a relatively thick coating of a cellulose ether soluble in the said volatile solvent; and stripping the compositely coated sheet from the polished surface.

4. The method which includes: depositing a uniform layer of a solution of an organo-soluble ethyl cellulose in a volatile solvent on a polished metal surface in amount sufficient to form a relatively thin film thereon upon evaporation of the solvent; partially drying the solution on the polished surface; superposing and pressing thereon a dry coated face of a flexible sheet coated on at least one side with a relatively thick coating of an organo-soluble ethyl cellulose soluble in the said volatile solvent; and stripping the compositely coated sheet from the polished surface.

5. The method which includes: depositing a uniform layer of a solution of an organo-soluble ethyl cellulose in a volatile solvent on the polished face of a heated rotating drum in amount sufficient to form a relatively thin film thereon upon evaporation of the solvent; partially drying the solution on the drum face; superposing and pressing thereon a dry coated face of a flexible paper sheet coated on at least one side with a relatively thick coating of an organo-soluble ethyl cellulose soluble in the said volatile solvent; stripping the compositely coated paper sheet from the drum face; and drying the compositely coated sheet.

6. The method which includes: depositing a uniform layer of a solution of an organo-soluble ethyl cellulose in a volatile solvent on the polished face of a heated rotating drum in amount sufficient to form a relatively thin film thereon upon evaporation of the solvent; partially drying the solution on the drum face; superposing and pressing thereon a dry coated face of a flexible paper sheet coated on at least one side with a relatively thick coating of an organo-soluble ethyl cellulose soluble in the said volatile solvent; reducing the proportion of said volatile solvent in the composite coating to from 3 per cent to 20 per cent of the weight thereof; and stripping the compositely coated paper sheet from the drum face.

7. The method which includes: depositing a uniform layer of a solution of organo-soluble ethyl cellulose in a volatile solvent on the polished face of a heated rotating drum in amount sufficient to form a film from 0.05 to 2.0 mils in thickness thereon upon evaporation of the solvent; partially drying the solution on the drum face; superposing and pressing thereon a dry coated face of a flexible paper sheet coated on at least one side with a coating from 3 to 8 mils in thickness of organo-soluble ethyl cellulose soluble in said volatile solvent; reducing the proportion of said volatile solvent in the composite coating to from 3 per cent to 20 per cent of the weight thereof; stripping the compositely coated paper sheet from the drum face; and drying the coated paper sheet.

WILLIAM R. COLLINGS.